



US005338379A

**United States Patent** [19]**Kelly**[11] **Patent Number:** **5,338,379**[45] **Date of Patent:** **Aug. 16, 1994****[54] TANTALUM-CONTAINING SUPERALLOYS**

[75] Inventor: Thomas J. Kelly, Cincinnati, Ohio

[73] Assignee: General Electric Company, Cincinnati, Ohio

[21] Appl. No.: 992,340

[22] Filed: Dec. 17, 1992

246082 11/1987 European Pat. Off. .

2220589 10/1974 France .

2328544 5/1977 France .

1052561 10/1966 United Kingdom .

1260982 1/1972 United Kingdom .

1011785 10/1975 United Kingdom .

1409628 10/1975 United Kingdom .

1471053 4/1977 United Kingdom .

1381859 5/1977 United Kingdom .

2152075A 7/1985 United Kingdom .

2191505 12/1987 United Kingdom .

**Related U.S. Application Data**

[60] Division of Ser. No. 658,417, Feb. 19, 1991, Pat. No. 5,207,846, which is a continuation-in-part of Ser. No. 335,353, Apr. 10, 1989, abandoned.

[51] **Int. Cl.<sup>5</sup>** ..... **C22C 19/05**[52] **U.S. Cl.** ..... **148/410; 148/419;**  
148/428; 148/675[58] **Field of Search** ..... 148/410, 428, 419, 675,  
148/555, 405**[56] References Cited****U.S. PATENT DOCUMENTS**3,668,023 6/1972 Kotval ..... 148/32.5  
4,981,644 1/1991 Chang ..... 420/442**FOREIGN PATENT DOCUMENTS**208645A3 1/1982 European Pat. Off. .  
225837 6/1987 European Pat. Off. .*Primary Examiner*—Richard O. Dean*Assistant Examiner*—Margery S. Phipps*Attorney, Agent, or Firm*—Jerome C. Squillaro; David L. Narciso**[57] ABSTRACT**

Nickel base superalloys which contain niobium (columbium) to promote gamma double prime strengthening are improved by replacing the niobium with tantalum on an atom-for-atom basis and then heat treating the new alloy at temperatures in excess of those conventionally used for superalloys which include niobium. The resultant tantalum-bearing alloys are found to exhibit increased strength and greater phase stability than corresponding niobium-bearing alloys.

**1 Claim, 1 Drawing Sheet****Effect of Iron on Ta718 Ultimate Strength**



Figure 1

## TANTALUM-CONTAINING SUPERALLOYS

This application is a divisional of 07/658,417 filed Feb. 19, 1991, now U.S. Pat. No. 5,207,846, which is a continuation-in-part of application Ser. No. 07/335,353 dated Apr. 19, 1989.

## BACKGROUND OF THE INVENTION

## 1. Field of the Invention

The present invention relates to improved nickel base alloys which have a particularly high combination of strength properties and ductility over the temperature range extending from about room temperature to approximately 1500° F. The improvement is provided by incorporating a substantial amount of tantalum in the alloy, generally as an atom-for-atom replacement for niobium, and then heat treating the alloy at very high temperatures for extended periods.

## 2. Description of the Prior Art

Prior art nickel-base superalloys while steadily being improved, have disadvantages either from a standpoint of strength or ductility, particularly at elevated temperatures, i.e., above about 1200° F. These alloys are generally based upon nickel in combination with one or more of chromium, iron, and cobalt. In addition, they may contain a variety of elements in a large number of combinations to produce desired effects. Some of the elements which have been utilized in nickel-base superalloys to provide or improve one or more of the following properties are: strength (Mo, Ta, W, Re), oxidation resistance (Cr, Al), phase stability (Ni) or increased volume fractions of favorable secondary precipitates (Co). Other elements are added to form hardening precipitates such as gamma prime (Al, Ti) and gamma double prime (Cb). Minor elements (C, B) are added to form carbides and borides and others (Ce, Mg) are added for purposes of tramp element control. Some elements (B, Zr, Hf) also are added to promote favorable grain boundary effects. Many elements (e.g., Co, Mo, W, Cr), although added for their favorable alloying qualities, can participate, in some circumstances, in the formation of undesirable phases (e.g., sigma, mu, Laves).

Gamma double prime is generally considered to be a body centered tetragonal ordered  $Ni_3Nb$  strengthening precipitate which is formed when niobium is present in nickel-base superalloys. A superalloy in which gamma double prime strengthening occurs is Inconel 718 which is within the scope of U.S. Pat. No. 3,046,108 (Eiselstein). Eiselstein teaches that the alloy must contain about 4 to about 8 weight percent columbium and that the columbium in the alloy may be replaced in part with tantalum in an amount of up to 4% of the alloy. In partially replacing the columbium content of the alloy with tantalum, Eiselstein teaches that double the weight of tantalum should be used to obtain the same effect on properties. He also teaches that only tantalum-free alloys and/or alloys wherein not more than 50% of the columbium is replaced by tantalum are notch-ductile at elevated temperatures. Eiselstein thus teaches that tantalum and niobium act the same in nickel-based alloys provided that only a limited amount of tantalum is present.

The gamma double prime phase is not normally a stable phase since it can convert to gamma prime or to delta on extended exposure to elevated temperatures. Alloys hardened with gamma double prime achieve

high tensile strength and very good creep rupture properties at lower temperatures, but the conversion of gamma double prime to gamma prime or delta above about 1250° F. causes a sharp reduction of strength. 5 (Donachie, M. J., "Relationship of Properties to Microstructure in Superalloys" in Superalloys Source Book, American Society for Metals, 1984).

## SUMMARY OF THE INVENTION

10 It has now been discovered that tantalum does not act the same as niobium in nickel base superalloys. Rather, tantalum has been found to produce an alloy which has greater phase stability and different phase relationships than the corresponding niobium containing alloy. This 15 difference in phase stability makes the Ta containing alloys much stronger to much higher temperatures than Nb containing alloys. In addition, the gamma double prime in the alloys of the invention does not readily convert to delta phase as occurs in niobium-bearing 20 counterpart alloys.

The present invention particularly contemplates a nickel base alloy which comprises at least about 30 weight percent nickel, about 8 to about 16 weight percent tantalum and which is substantially niobium-free. 25 Additional elements contained in the alloy are primarily selected from the group consisting of chromium, iron, cobalt, molybdenum, titanium, zirconium, tungsten, hafnium, aluminum, boron, and carbon and combinations thereof. In addition, other elements such as manganese, silicon, phosphorus, sulfur, lead, bismuth, tellurium, selenium, niobium and silver may also be present as incidental impurities.

30 The invention further extends broadly to the method for improving the high temperature strength properties of niobium-bearing nickel base superalloys by replacing substantially all of the niobium contained therein with tantalum on an atom-for-atom basis.

The invention also comprehends a method for improving the high temperature strength properties of the tantalum-bearing nickel base superalloys of the invention by heat treatments at higher temperatures and for longer duration than those used for their niobium-bearing 40 counterparts.

## BRIEF DESCRIPTION OF THE DRAWINGS

FIG. 1 is a graph representing a plot of the ultimate tensile strength vs. iron content of the alloys of the present invention.

## DESCRIPTION OF THE PREFERRED EMBODIMENT

The alloys of the present invention contain at least about 30% nickel (all percents expressed herein and in the claims are by weight unless otherwise specified) and about 8 to about 16% tantalum. The balance of the alloy will consist of other elements which are conventionally alloyed with nickel to form superalloys such as elements selected from the group consisting of chromium, iron, cobalt, molybdenum, titanium, zirconium, tungsten, hafnium, aluminum, boron, carbon and combinations thereof. Further, other elements such as manganese, silicon, phosphorus, sulfur, lead, bismuth, tellurium, selenium, and silver may also be found in the alloy as 55 incidental impurities. These alloys will be substantially niobium-free, i.e., they will contain less than about 1%, preferably less than 0.5%, and most preferably less than about 0.1% Nb.



TABLE I-continued

| Cast Ta 718 <sup>1,3</sup> |      |      |      | Cast Nb 718 <sup>1</sup> |    | Cast Ta 718 <sup>2,4</sup> |      |   |
|----------------------------|------|------|------|--------------------------|----|----------------------------|------|---|
| RT                         | 1200 | 1300 | RT   | 1200                     | RT | 1200                       | 1400 |   |
| % RA                       | 29.1 | 22.5 | 21.5 | 29                       | 29 | 18                         | 8    | 6 |

<sup>1</sup>2000° F./1 hr; 2050 hip/14.7ksi/3 hr; 1925/1 hr; 1350/8 hr; 1150/8 hr.<sup>2</sup>2000° F./1 hr; 2050 hip/14.7ksi/3 hr; 1925/1 hr; 1600/2 hr; 1350/8 hr.<sup>3</sup>Average of 2 specimens<sup>4</sup>One specimen

As may be noted from Table I, the tantalum-bearing 718 type superalloy showed improved elevated temperature strength properties over its niobium-bearing counterpart and these properties were even further improved by the use of the preferred heat treatment.

### EXAMPLE II

The procedure of Example I was repeated with an alloy whose composition was 36.6% nickel, 36.6% iron, 17.7% cobalt, 9.1% tantalum, and 45 ppm boron. The corresponding conventional alloy in which the tantalum is replaced with niobium on an atom for atom basis, i.e. the niobium content is 4.5%, was also prepared for comparison purposes. The alloys are evaluated for mechanical properties as in Example I. The results are:

TABLE II

|                                 | Cast Ta Alloy |          | Cast Nb Alloy |          |
|---------------------------------|---------------|----------|---------------|----------|
|                                 | R.T.          | 1200° F. | R.T.          | 1200° F. |
| Ultimate tensile strength (KSI) | 182.5         | 141.8    | 135           | 108      |
| 0.2% Yield strength (KSI)       | 159.4         | 128.6    | 120           | 89       |
| % Elongation                    | 4.5           | 3.0      | 4.0           | 7.0      |
| % Reduction in area             | 6.5           | 6.5      | 7.0           | 13.0     |

As is evident, the tantalum-bearing alloy of the present invention exhibits substantially increased ultimate tensile and yield strengths, reduced reduction in area, and similar elongation as compared to the same alloy containing niobium.

Evaluations of the various alloys again demonstrate the superiority of the tantalum-bearing alloy of this invention as compared to the comparable niobium-bearing alloy.

### EXAMPLE III

Although the conventional 718 alloy of Example I is highly resistant to strain-age cracking during weld stress relief, the alloy can be susceptible to both liquation cracking in the weld heat-affected-zone (HAZ) and, under conditions of high restraint, solidification cracking in the weld fusion zone. To evaluate the effect of the tantalum for niobium substitution of the present invention, the alloy formation steps of Example I are repeated to produce cast-to-size weldability test specimens 5 mm in thickness. Prior to weldability testing all specimens were heat treated in vacuum at 2000° F. for one hour and cooled to 1200° F. in twenty minutes. Spot Varestraint and Mini Varestraint weldability tests were utilized to evaluate HAZ liquification and fusion zone solidification cracking susceptibilities. In the Spot Varestraint test, strain is applied to a gas-tungsten-arc spot weld immediately after extinguishing the arc, thereby restricting cracking to the weld HAZ. During Mini Varestraint testing, straining occurs during the generation of a continuous gas tungsten-arc weld, with cracks forming primarily in the previously solidified fusion

zone. Total crack length is utilized as the quantitative measure of cracking susceptibility.

As shown in Table III, the tantalum-bearing alloy exhibits the lowest susceptibility to weld HAZ cracking over the entire range of strain levels tested, i.e. 0.25 to 3% augmented strain, by the Spot Varestraint test.

TABLE III

| Strain | Cracks | Cast Alloy 718 |      | Cast Ta 718 |      |
|--------|--------|----------------|------|-------------|------|
|        |        | TCL            | MCL  | Cracks      | TCL  |
| 0.29%  | 24     | .422           | .032 | 12          | .214 |
| 0.29%  | 26     | .493           | .033 | 12          | .240 |
| 1.16%  | 33     | .671           | .040 | 19          | .391 |
| 1.16%  | 35     | .775           | .040 | 20          | .462 |
| 2.9%   | 42     | 1.008          | .055 | 30          | .664 |
| 2.9%   | 48     | 1.108          | .053 | 30          | .669 |

Cracks: number of cracks per weld

TCL: Total Crack Length

MCL: Maximum Crack Length

### EXAMPLE IV

Cast tantalum-containing nickel base superalloys having the chemical compositions listed in Table IV in accordance with the methods of Example 1.

TABLE IV

| Alloy | Fe    | Al   | Ti   | Ta   | Cr    | Mo   | B      | C      |
|-------|-------|------|------|------|-------|------|--------|--------|
| HTD-1 | 12.98 | 0.49 | 1.55 | 8.97 | 19.08 | 2.98 | 0.0034 | 0.0234 |
| HTD-2 | 18.39 | 0.99 | 2.02 | 9.01 | 18.20 | 3.00 | 0.004  | 0.019  |
| HTD-3 | 13.34 | 0.99 | 1.03 | 9.05 | 18.15 | 3.09 | 0.0035 | 0.02   |
| HTD-4 | 18.02 | 1.01 | 1.53 | 9.11 | 18.07 | 2.98 | 0.0039 | 0.02   |
| HTD-5 | 18.29 | 0.50 | 2.04 | 9.02 | 18.29 | 2.99 | 0.0040 | 0.02   |
| HTD-6 | 13.36 | 0.50 | 1.03 | 9.02 | 18.12 | 3.06 | 0.0035 | 0.02   |
| HTD-7 | 20.44 | 0.54 | 0.91 | 8.96 | 18.90 | 3.28 | 0.004  | 0.06   |

\*for HTD

The room temperature mechanical properties of each of the alloys is provided in Table V.

TABLE V

| Alloy | UTS (KSI) | RA (%) | TCL** |
|-------|-----------|--------|-------|
| HTD-1 | 157.9     | 8.2    | 0.432 |
| HTD-2 | 131.6     | 4.4    | 0.496 |
| HTD-3 | 150.3     | 7.9    | 0.336 |
| HTD-4 | 132.3     | 7.2    | 0.872 |
| HTD-5 | 142.3     | 7.2    | 0.872 |
| HTD-6 | 154.7     | 8.0    | 0.448 |
| HTD-7 | ***       | ***    | ***   |

\*\*total crack length measured (inches)

\*\*\*not available

The graph of he iron content is shown in FIG. 1 The data indicate that the iron content is influential in ductility and strength. Additionally the iron content affects weldability, as indicated by total crack length. From the data, the best combination of properties is obtainable with an iron content of about 11% to about 15%.

The preferred cast nickel-base tantalum containing alloy prepared in accordance with the methods of Example I has an alloy composition, within melt tolerances, consisting essentially of about 11.34-15.34% iron, about 16.15-20.15% chromium, about 2.79-3.39% molybdenum, about 8.81-9.31% tantalum, about 0.73-1.33% titanium, about 0.69-1.29% aluminum, about 0.003-0.007% boron, about 0.05-0.15% carbon and the balance essentially nickel. The nominal composition of this alloy consists essentially of about 13.34% iron, about 18.15% chromium, about 3.09% molybdenum, about 9.11% tantalum, about 1.03% titanium, about 1.0% aluminum, bout 0.0035% boron, about 0.1% carbon and the balance essentially nickel.

The elevated temperature tests of the alloys of this nominal chemistry are provided in Table VI.

TABLE VI

| Temp °F. | UTS (KSI) | YS (KSI) | TA (%) | % Elong. |
|----------|-----------|----------|--------|----------|
| 1200     | 135.8     | 121.2    | 15.7   | 4.8      |
| 1400     | 128.9     | 116.1    | 3.5    | 3.0      |
| 1600     | 82.4      | 82.4     | 11.8   | 1.6      |

In addition to these tests, notch-rupture/stress rupture tests at 65 ksi and creep tests at 25 ksi were run at 1400° F. for 100 hours and 1000 hours respectively. The alloy of the preferred composition showed no susceptibility to stress-rupture failure at the stress levels and temperatures of test. The alloy also showed no susceptibility to creep failure at the stress levels and temperatures of test as indicated by zero strain measurement.

The unexpectedly superior combination of properties of the alloys of the preferred embodiment make it particularly suitable for applications in which these properties are required even after a weld repair.

The alloys of the preferred composition are characterized by a microstructure having a uniform gamma prime and gamma double prime distribution of a size which produces a reasonable strengthening effect. The gamma prime and gamma double prime are much more

uniformly distributed throughout the dendrite core and interstices than in conventional cast 718 alloys.

Although the present invention has been described in connection with specific examples and embodiments, it will be understood by those skilled in the arts involved that the present invention is capable of modification without departing from its spirit and scope as represented by the appended claims.

What is claimed is:

10. 1. A weldable, cast nickel base superalloy which consists essentially of, in weight percent, about 13.34% iron, about 18.15% chromium, about 3.09% molybdenum, about 9.11% tantalum, about 1.03% titanium, about 1.0% aluminum, about 0.0035% boron, about 0.1% carbon, and the balance essentially nickel, the superalloy being characterized by a microstructure having a uniform distribution of gamma prime and gamma double prime precipitates, the gamma prime and gamma double prime precipitates having been formed with a gamma matrix by first heating the cast alloy to a temperature of about 2000° F. for about 1 hour, heating the alloy at a temperature of about 2050° F. for about 3 to about 5 hours, then cooling the alloy to a temperature of about 1925° F. and holding it at about 1925° F. for about 4 hours, cooling to a first aging temperature of about 1600° F. and aging for about 2 hours and optionally cooling to a second aging temperature of about 1350° F. and aging for about 8 hours.

\* \* \* \* \*

30

35

40

45

50

55

60

65